

## 1

3,457,030

**METHOD OF INHIBITING CORROSION**

Mark T. Atwood, Donald R. Napier, and Donald H. Oertle, Ponca City, Okla., assignors to Continental Oil Company, Ponca City, Okla., a corporation of Delaware  
 No Drawing. Filed Dec. 29, 1965, Ser. No. 517,460  
 Int. Cl. C23f 11/16, 11/04

U.S. Cl. 21—2.7

10 Claims

**ABSTRACT OF THE DISCLOSURE**

Use of certain thiuronium compounds to inhibit corrosion of ferrous metals exposed to aqueous systems containing hydrochloric acid, hydrogen sulfide, carbon dioxide or mixtures thereof. An illustrative thiuronium compound is bis (isothiureidomethyl) dodecylbenzene dihydrochloride.

The present invention relates to a method of inhibiting corrosion of ferrous metals exposed to aqueous systems containing hydrochloric acid, hydrogen sulfide, carbon dioxide or mixtures thereof. More particularly, the present invention relates to a method of inhibiting corrosion of the aforementioned type through the use of certain thiuronium compounds.

It is well known that exposure of ferrous metals to aqueous systems results in corrosion of the metals. This is particularly true when the aqueous systems contain appreciable amounts of hydrogen chloride, hydrogen sulfide, carbon dioxide, or mixture of these materials. One means of alleviating this type of corrosion is by adding to the aqueous systems various chemical compounds. Many chemicals are known which inhibit the corrosion of ferrous metals which are exposed to aqueous systems containing hydrogen chloride, hydrogen sulfide, or carbon dioxide. It is highly desirable for those working in this field to have available chemical compounds which are effective at low concentrations (e.g., less than 100 parts per million). It is also highly desirable for those working in this field to have available a number of chemical compounds which are suitable as inhibitors. This is particularly true, since the economics may change and a corrosion inhibitor, once considered uneconomical, is then economical to use. Also, a choice of inhibitors give those working in this field a choice of suppliers.

It is an object of the present invention to provide an improvement in the means of inhibiting corrosion through the use of certain corrosion inhibitors of improved efficiency.

It is another object of the invention to provide an improved method of inhibiting corrosion of ferrous metals in contact with aqueous systems containing hydrochloric acid, hydrogen sulfide, carbon dioxide or mixtures thereof.

It is a particular object of the invention to inhibit corrosion of the type described above through the use of certain thiuronium compounds.

Broadly stated the present invention relates to a method of inhibiting corrosion of ferrous metals in contact with aqueous systems containing hydrogen sulfide, hydrogen chloride, carbon dioxide, or mixtures thereof, wherein the method comprises adding to the aqueous system, a corrosion-inhibiting amount of a thiuronium compound represented by the formula



## 2

wherein R is an alkyl group, either branched or straight chain, containing from 6 to 18 carbon atoms, wherein A is either hydrogen or a methyl group, wherein X is a halogen, which, preferably, is chlorine, and wherein n is a number of from about 1 to about 2.8.

Preferably, the method of our invention uses a thiuronium compound represented by the formula



wherein R is an alkyl group, either branched or straight chain, containing from about 10 to about 18 carbon atoms, preferably from about 10 to about 14 carbon atoms, wherein A is either hydrogen or a methyl group, wherein X is a halogen, which, preferably, is chlorine, and wherein n is a number of from about 1.4 to about 2.8, preferably from about 1.6 to about 2.4. For convenience, compounds wherein n is from about 1.4 to about 2.8 are referred to as "bis" thiuronium compounds.

More preferably, the method of our invention relates to a method of inhibiting corrosion of ferrous metals in contact with aqueous systems containing hydrogen sulfide, wherein the method comprises adding to the aqueous system a corrosion-inhibiting amount of a "bis" thiuronium compound as described immediately above.

Examples of suitable thiuronium compounds for use in the method of our invention have the formula



wherein R, A, X and n are as follows:

| R                                            | A               | X  | n   |
|----------------------------------------------|-----------------|----|-----|
| n-C <sub>6</sub> -C <sub>18</sub> (mixed)    | H               | Cl | 1.0 |
| br-C <sub>6</sub> -C <sub>18</sub> (mixed)   | H               | Cl | 1.2 |
| n-C <sub>6</sub> -C <sub>18</sub> (mixed)    | H               | Br | 1.4 |
| br-C <sub>6</sub> -C <sub>18</sub> (mixed)   | H               | I  | 1.6 |
| n-C <sub>6</sub> -C <sub>18</sub> (mixed)    | CH <sub>3</sub> | Cl | 1.8 |
| br-C <sub>6</sub> -C <sub>18</sub> (mixed)   | CH <sub>3</sub> | Cl | 2.0 |
| n-C <sub>6</sub> -C <sub>1</sub> (mixed)     | CH <sub>3</sub> | Br | 2.2 |
| br-C <sub>6</sub> -C <sub>18</sub> (mixed)   | CH <sub>3</sub> | Br | 2.4 |
| n-C <sub>6</sub>                             | H               | Cl | 2.6 |
| n-C <sub>8</sub>                             | H               | Cl | 2.8 |
| n-C <sub>10</sub>                            | H               | Cl | 2.6 |
| n-C <sub>12</sub>                            | H               | Cl | 2.4 |
| n-C <sub>14</sub>                            | H               | Cl | 2.2 |
| n-C <sub>16</sub>                            | CH <sub>3</sub> | Cl | 2.0 |
| n-C <sub>8</sub>                             | CH <sub>3</sub> | I  | 1.8 |
| n-C <sub>10</sub>                            | CH <sub>3</sub> | Cl | 1.6 |
| n-C <sub>12</sub>                            | CH <sub>3</sub> | Cl | 1.4 |
| n-C <sub>14</sub>                            | CH <sub>3</sub> | Cl | 1.2 |
| n-C <sub>6</sub> -C <sub>18</sub> (mixed)    | H               | Cl | 1.4 |
| br-C <sub>6</sub> -C <sub>18</sub> (mixed)   | H               | Cl | 1.6 |
| n-C <sub>6</sub> -C <sub>18</sub>            | H               | Br | 1.8 |
| br-C <sub>6</sub> -C <sub>18</sub> (mixed)   | H               | Br | 2.0 |
| n-C <sub>6</sub> -C <sub>18</sub> (mixed)    | CH <sub>3</sub> | Cl | 2.2 |
| br-C <sub>6</sub> -C <sub>18</sub> (mixed)   | CH <sub>3</sub> | Cl | 2.4 |
| n-C <sub>6</sub> -C <sub>1</sub> (mixed)     | CH <sub>3</sub> | Br | 2.6 |
| br-C <sub>6</sub> -C <sub>18</sub> (mixed)   | CH <sub>3</sub> | Br | 2.8 |
| n-C <sub>6</sub>                             | H               | Cl | 1.4 |
| n-C <sub>8</sub>                             | H               | Cl | 1.6 |
| n-C <sub>10</sub>                            | H               | Cl | 1.8 |
| n-C <sub>12</sub>                            | H               | Cl | 2.0 |
| n-C <sub>14</sub>                            | H               | Cl | 2.0 |
| n-C <sub>6</sub>                             | CH <sub>3</sub> | Cl | 2.4 |
| n-C <sub>8</sub>                             | CH <sub>3</sub> | Cl | 2.6 |
| n-C <sub>10</sub>                            | CH <sub>3</sub> | Cl | 2.8 |
| n-C <sub>12</sub>                            | CH <sub>3</sub> | Cl | 1.8 |
| n-C <sub>14</sub>                            | CH <sub>3</sub> | Cl | 1.6 |
| n-C <sub>10</sub> -C <sub>18</sub> (mixed)*  | H               | Cl | 1.6 |
| br-C <sub>10</sub> -C <sub>18</sub> (mixed)* | H               | Cl | 1.8 |

| R                                            | A               | X  | n   |
|----------------------------------------------|-----------------|----|-----|
| n-C <sub>10</sub> -C <sub>14</sub> (mixed)*  | H               | I  | 2.0 |
| br-C <sub>10</sub> -C <sub>14</sub> (mixed)* | H               | Cl | 2.2 |
| n-C <sub>10</sub> -C <sub>18</sub> (mixed)*  | CH <sub>3</sub> | Cl | 2.4 |
| br-C <sub>10</sub> -C <sub>18</sub> (mixed)* | CH <sub>3</sub> | Cl | 2.6 |
| n-C <sub>10</sub> -C <sub>14</sub> (mixed)*  | CH <sub>3</sub> | Cl | 2.8 |
| br-C <sub>10</sub> -C <sub>14</sub> (mixed)* | CH <sub>3</sub> | Cl | 1.4 |
| n-C <sub>10</sub> -C <sub>18</sub> (mixed)*  | H               | Br | 1.6 |
| br-C <sub>10</sub> -C <sub>18</sub> (mixed)* | H               | Br | 1.8 |
| n-C <sub>10</sub> -C <sub>14</sub> (mixed)*  | H               | Br | 2.0 |
| br-C <sub>10</sub> -C <sub>11</sub> (mixed)* | H               | Br | 2.2 |
| n-C <sub>10</sub> -C <sub>18</sub> (mixed)*  | CH <sub>3</sub> | Br | 2.4 |
| br-C <sub>10</sub> -C <sub>18</sub> (mixed)* | CH <sub>3</sub> | I  | 2.2 |
| n-C <sub>10</sub> -C <sub>14</sub> (mixed)*  | CH <sub>3</sub> | Br | 2.0 |
| br-C <sub>10</sub> -C <sub>14</sub> (mixed)* | CH <sub>3</sub> | Br | 1.8 |
| n-C <sub>10</sub>                            | H               | Cl | 1.7 |
| n-C <sub>12</sub> *                          | H               | Cl | 1.9 |
| n-C <sub>14</sub> *                          | H               | Cl | 2.1 |
| n-C <sub>16</sub> *                          | H               | Cl | 2.3 |
| n-C <sub>18</sub> *                          | H               | Cl | 2.1 |
| br-C <sub>10</sub> *                         | H               | Cl | 1.9 |
| br-C <sub>12</sub> *                         | H               | Cl | 1.7 |
| br-C <sub>14</sub> *                         | H               | Cl | 1.9 |
| br-C <sub>16</sub> *                         | H               | Cl | 2.1 |
| br-C <sub>18</sub> *                         | H               | Cl | 2.3 |
| n-C <sub>10</sub> *                          | CH <sub>3</sub> | Cl | 2.0 |
| n-C <sub>12</sub> *                          | CH <sub>3</sub> | Cl | 2.2 |
| n-C <sub>14</sub> *                          | CH <sub>3</sub> | Cl | 2.4 |
| n-C <sub>16</sub> *                          | CH <sub>3</sub> | Cl | 2.0 |
| n-C <sub>18</sub> *                          | CH <sub>3</sub> | Cl | 2.2 |
| br-C <sub>10</sub> *                         | CH <sub>3</sub> | Cl | 2.4 |
| br-C <sub>12</sub> *                         | CH <sub>3</sub> | Cl | 2.1 |
| br-C <sub>14</sub> *                         | CH <sub>3</sub> | Cl | 2.3 |
| br-C <sub>16</sub> *                         | CH <sub>3</sub> | Cl | 2.0 |
| br-C <sub>18</sub> *                         | CH <sub>3</sub> | Cl | 2.2 |
| n-C <sub>10</sub> *                          | H               | Br | 2.1 |
| n-C <sub>12</sub> *                          | H               | Br | 2.3 |
| n-C <sub>14</sub> *                          | H               | Br | 1.8 |
| n-C <sub>16</sub> *                          | H               | Br | 1.6 |
| n-C <sub>18</sub> *                          | H               | Br | 1.8 |
| br-C <sub>10</sub> *                         | H               | Br | 1.7 |
| br-C <sub>12</sub> *                         | H               | Br | 1.9 |
| br-C <sub>14</sub> *                         | H               | Br | 2.1 |
| br-C <sub>16</sub> *                         | H               | Br | 2.3 |
| br-C <sub>18</sub> *                         | H               | Br | 2.0 |
| n-C <sub>10</sub> *                          | CH <sub>3</sub> | Br | 2.0 |
| n-C <sub>12</sub> *                          | CH <sub>3</sub> | Br | 2.2 |
| n-C <sub>14</sub> *                          | CH <sub>3</sub> | Br | 2.4 |
| n-C <sub>16</sub> *                          | CH <sub>3</sub> | Br | 1.6 |
| n-C <sub>18</sub> *                          | CH <sub>3</sub> | Br | 1.8 |
| br-C <sub>10</sub> *                         | CH <sub>3</sub> | Br | 1.6 |
| br-C <sub>12</sub> *                         | CH <sub>3</sub> | Br | 1.8 |
| br-C <sub>14</sub> *                         | CH <sub>3</sub> | Br | 2.0 |
| br-C <sub>16</sub> *                         | CH <sub>3</sub> | Br | 2.2 |
| br-C <sub>18</sub> *                         | CH <sub>3</sub> | Br | 2.5 |

The asterisk indicates that these particular compounds are preferred. The term "n" refers to straight chain; the term "br" to branched chain. The term "mixed" means that alkyl groups of varying chain length are present.

Inasmuch as the alkylaromatic portion of the thiuronium compounds of our invention is an important feature of our invention, this will be described in considerable detail. The aromatic radical of the compounds of our invention is derived from either benzene or toluene, but preferably is derived from benzene. The long chain alkyl group of the alkylaromatic portion of the thiuronium compounds of our invention can be either straight or branched chain, and contains from about 6 to about 18 carbon atoms. Usually, the alkyl group contains from 10 to 18 carbon atoms, but preferably contains from 10 to 14 carbon atoms. The thiuronium compounds can be derived from a single alkylaromatic compound (e.g., hexylbenzene, octylbenzene, decylbenzene, etc.). More usually, the thiuronium compounds are derived from mixtures of alkylaromatic hydrocarbons containing alkyl groups of varying lengths, as hereinbefore defined. In fact, the more suitable commercially available alkylaromatic hydrocarbons are mixtures.

An example of a particularly suitable commercially available alkylaromatic hydrocarbon which can be used to prepare the corrosion inhibitors of our invention is a material which is known to the trade as dodecylbenzene. Dodecylbenzene is available under the trade name of "Neolene" 400 from Continental Oil Company. In a typical process dodecylbenzene is prepared by first polymerizing propylene to produce a mixture of olefins which are predominantly C<sub>12</sub> (dodecene). Benzene is then alkylated with the dodecene to produce dodecylbenzene. The preparation of dodecylbenzene is described more completely in U.S. Patent 2,941,015 to Robert R. Kylander, 75

which patent is made a part of this specification. A typical sample of dodecylbenzene has the following properties:

| Distillation range, ° F.: |                                                       |
|---------------------------|-------------------------------------------------------|
| 5                         | I.B.P. ----- 535                                      |
|                           | 5% ----- 545                                          |
|                           | 10% ----- 550                                         |
|                           | 50% ----- 560                                         |
|                           | 90% ----- 580                                         |
| 10                        | 97% ----- 592                                         |
|                           | F.B.P. ----- 603                                      |
|                           | Percent recovery ----- 99                             |
|                           | Specific gravity, 60° F. ----- 0.875                  |
|                           | Molecular weight <sup>1</sup> ----- 237               |
|                           | Aniline point <sup>2</sup> ----- 48.5                 |
|                           | Bromine No. <sup>3</sup> ----- 0.12                   |
|                           | Saybolt color <sup>4</sup> ----- 29                   |
|                           | Refractive index, 25° C. ----- 1.4885                 |
| 20                        | Appearance, clear and water white                     |
|                           | Flash point (closed cup), ° F. <sup>5</sup> ----- 260 |
|                           | Viscosity, centipoises:                               |
|                           | 68° F. ----- 14                                       |
|                           | 32° F. ----- 37                                       |

<sup>1</sup> Cryogenic method using benzene.

<sup>2</sup> ASTM D-611.

<sup>3</sup> ASTM D-1159.

<sup>4</sup> ASTM D-156.

<sup>5</sup> ASTM D-56.

It is generally known that the alkyl group in dodecylbenzene is branched chain. More recently, in order to produce detergents which are less resistant to attack by bacteria, straight chain alkylaromatic hydrocarbons, similar to dodecylbenzene, have been prepared. These materials constitute a class of materials which, when sulfonated, are known in industry as biodegradable detergents. It is to be understood that any of the n-alkylaromatic hydrocarbons which are used in preparing biodegradable detergents and having at least 10 carbon atoms in the alkyl group can be used to prepare the corrosion inhibitors of our invention.

The preparation of a particularly suitable n-alkylaromatic hydrocarbon for use in our invention is described in application Ser. No. 129,252, filed Aug. 4, 1961, and now abandoned, and having the same assignee as the present application. For reason of convenience, this application is made a part of the present application. Briefly, application Ser. No. 129,252 relates to a process of preparing a detergent alkylate wherein the process comprises the following steps, broadly stated: (a) separating a fraction of substantially straight chain C<sub>8</sub>-C<sub>18</sub> hydrocarbons from a petroleum distillate substantially free of olefins and containing said straight chain hydrocarbons together with non-straight chain hydrocarbons, (b) chlorinating said fraction to the extent whereby between about 10 and about 35 mole percent of the straight chain hydrocarbons present are substantially only monochlorinated, (c) alkylating an aromatic compound, selected from the group consisting of benzene, a lower alkyl substituted benzene and mixtures thereof, with the chlorination product of step (b) in the presence of an alkylation catalyst.

n-Alkylaromatic hydrocarbons of the aforementioned type are available under the trademarks "Nalkylene" 500 and "Nalkylenes" 600 from Continental Oil Company. These materials have the following typical properties:

#### "NALKYLENE" 500

| Test                        | Typical Value    | Test Method  |
|-----------------------------|------------------|--------------|
| Boiling range (° F.)        | 535-595          | ASTM D-447.  |
| Bromine No.                 | 0.05 max.        | ASTM D-1158. |
| Average molecular weight    | 231-241          | Mass spec.   |
| Color—Saybolt               | +25              |              |
| Specific gravity (20/20)    | 0.85-0.87        | ASTM D-287.  |
| Viscosity (Saybolt seconds) | 40-45 at 100° F. | ASTM 88-44.  |

## "NALKYLENE" 600

|                             |                  |              |
|-----------------------------|------------------|--------------|
| Boiling range (° F.):       |                  |              |
| 5%                          | 580-590          | ASTM D-447.  |
| 95%                         | 600-615          |              |
| Bromine No.                 | 0.05 max         | P.M. No. 21. |
| Average molecular weight    | 255-264          | Mass spec.   |
| Color—Saybolt               | 25 min.          | P.M. No. 20. |
| Specific gravity            | 0.85-0.87        | ASTM D-287.  |
| Viscosity (Saybolt seconds) | 40-46 at 100° F. | ASTM 88-44.  |

Still another suitable alkylaromatic hydrocarbon for use in preparing the corrosion inhibitor of our invention is a byproduct of the production of a material which we refer to as "dimer alkylate." "Dimer alkylate" has branched-chain alkyl groups, as does dodecylbenzene. Briefly described, dimer alkylate is prepared by the following steps:

- (1) dimerization of a suitable feedstock, such as cat poly gasoline, and
- (2) alkylation of an aromatic hydrocarbon with the dimer formed in step (1).

The dimerization step uses a Friedel-Crafts alkylation sludge as a catalyst. This process is described in application Ser. No. 367,417, filed May 14, 1964, and having the same assignee as the present application. The fraction produced by the dimer alkylate process which is suitable for use in preparing the product of this invention is that having a boiling range of about 475 to about 600° F., preferably about 500 to about 590° F., as determined by ASTM procedure D-86.

## DESCRIPTION OF PREPARATION OF THIURONIUM COMPOUNDS

The first step in preparing the thiuronium compounds of our invention is the preparation of a halomethylated alkylaromatic hydrocarbon (preferably ("bis" chloromethylated alkylaromatic hydrocarbon). In one method these materials are prepared by using a chloromethylating agent which is formed by reacting formaldehyde or a compound which engenders formaldehyde with a chlorine-containing compound which will engender hydrogen chloride in the presence of an alcohol and sulfuric acid. In addition to chloromethylating agents it is possible to use halomethylating agents which contain other halogens, such as bromine or iodine, which are prepared in a similar manner.

Suitable chlorine-containing compounds which will engender hydrogen chloride under the conditions used herein include phosphorus trichloride, phosphorus pentachloride, sulfuric oxychloride, sulfurous oxychloride, and acyl chlorides such as acetyl chloride.

Suitable alcohols are the primary monatomic saturated aliphatic alcohols containing from 1 to 4 carbon atoms, such as, for example, methanol, ethanol, normal propanol and normal butanol.

The relative amounts of the various components of the chloromethylating reagent, and the amount of chloromethylating agent used in relation to the alkaryl hydrocarbon, are shown below.

|                                                      | Suitable<br>(moles) | Preferred<br>(moles) |
|------------------------------------------------------|---------------------|----------------------|
| Alkaryl hydrocarbon                                  | 1                   | 1                    |
| Formaldehyde                                         | 2.1-4.0             | 3.4-3.6              |
| Alcohol                                              | 2.1-4.0             | 3.2-3.4              |
| Chlorine-containing compound (e.g., $\text{PCl}_3$ ) | 1.0-3.0             | 1.1-1.3              |
| Sulfuric acid                                        | 2.6-6.0             | 4.0-5.0              |

The chloromethylation reaction is conducted at a temperature in the range of about 65 to about 80° C., preferably about 66 to about 68° C., and for a time in the range of from about 2 to about 10 hours, preferably from about 4 to about 6 hours.

Specifically, the chloromethylation procedure can be illustrated by the following procedure which shows the

preparation of a monohalomethylated alkylaromatic hydrocarbon: 200 grams of dodecylbenzene is treated with a chloromethylating mixture which has been prepared as follows: 42 grams of p-formaldehyde and 43 grams methyl alcohol are added to a 1-liter Morton flask which is equipped with a sealed stirrer, thermometer, and dropping funnel. The flask is placed in an ice bath and mixing is begun. Phosphorus trichloride (65.5 grams) is added dropwise from the funnel while maintaining a temperature between 29 and 32° C. After the chloride addition, the reaction mass is aged 10 minutes at the same temperature. One hundred seventy-five grams of 100 percent sulfuric acid is then added to the dropping funnel. The sulfuric acid is then added to the reaction mass at a rate to maintain the same temperature. This is followed by post-stirring for an additional 15 minutes. This reaction mass and the dodecylbenzene are combined and heated at 52-55° C. for 3 hours to produce the chloromethylated dodecylbenzene.

The preparation of the bis halomethylated alkylaromatic hydrocarbon is similar to the preceding, with the exception that 100 grams of alkylaromatic hydrocarbon is used and the time and temperature are 5 hours and 67° C., respectively.

With regard to the "bis" halomethylated products, they are mixtures of homologous products containing 1, 2 or 3 halomethyl groups. Moreover, the distribution of these products varies according to the type of alkylaromatic hydrocarbon employed. Thus, while the above-identified "Neolene" 400 and "Nalkylene" 500 exhibit approximately equal reactivity in a dihalomethylation process, the product of the former is essentially all "bis" derivative, whereas the product of the latter is more nearly a mixture of mono and tris derivatives.

The degree of halomethylation is the average of the number of halomethyl groups present. As indicated previously, for reason of convenience we refer to those compounds derived from materials having from about 1.4 to about 2.8 halomethyl groups, preferably from about 1.6 to about 2.4 halomethyl groups, as "bis" compounds.

The second step in the process of preparing the corrosion inhibitors of our invention comprises reacting the halomethylated alkylaromatic hydrocarbon with thiourea. The reaction is generally carried out in the presence of an inert volatile organic solvent (e.g., isopropanol). Since the reaction of the second step is well known to those skilled in the art, it is believed that further description is unnecessary.

The thiuronium compounds in some instances can suitably be used as corrosion inhibitors in concentrations as low as 2 parts per million (by weight) based on the aqueous solution in which it is used. More suitably, the thiuronium compounds are used in a concentration of at least 10 parts per million. Preferably, they are used in a concentration of at least 50 parts per million. The "bis" thiuronium compounds are more effective than the mono-thiuronium compound. In addition, the effectiveness of the "bis" thiuronium compounds varies slightly depending on the nature of the alkylaromatic portion.

In order to disclose the nature of the present invention still more clearly, the following illustrative examples will be given. It is to be understood that the invention is not to be limited to the specific conditions or details set forth in these examples except in so far as such limitations are specified in the appended claims.

## Example 1

Using the procedure described hereinbefore, and using commercial dodecylbenzene as the alkylaromatic hydrocarbon, the monothiuronium compound was prepared. (This material is referred to as Compound A in the table below.) Similarly, using hexylbenzene as the alkylaromatic hydrocarbon, the monothiuronium compound was prepared. (This material is referred to as Compound B in the table below.)



2. The method of claim 1 wherein the compound has the formula:



wherein R is an alkyl group containing from about 6 to about 18 carbon atoms, wherein A is selected from the group consisting of hydrogen and a methyl radical, and wherein X is a halogen.

3. The method of claim 1, wherein the compound has the formula:



wherein R is an alkyl group containing from about 10 to about 18 carbon atoms, wherein A is selected from the group consisting of hydrogen and a methyl radical, wherein X is a halogen and wherein n is a number of from about 1.4 to about 2.8.

4. The method of claim 3, characterized further in that X is chlorine.

5. The method of claim 4, characterized further in that n is a number of from about 1.6 to about 2.4.

6. The method of inhibiting corrosion of ferrous metal in contact with aqueous systems containing hydrogen sulfide, said method comprising adding to the aqueous system a corrosion inhibiting amount of a compound represented by the formula:



wherein R is an alkyl group containing from about 10 to about 18 carbon atoms, wherein A is selected from the group consisting of hydrogen and a methyl radical, wherein X is a halogen, and wherein n is a number of from about 1.4 to about 2.8.

7. The method of claim 6, characterized further in that X is chlorine.

8. The method of claim 7, characterized further in that n is a number of from about 1.6 to about 2.4.

9. The method of claim 8, characterized further in that R is an alkyl group containing from about 10 to about 14 carbon atoms.

10. The method of claim 9, characterized further in that A is hydrogen.

#### References Cited

##### UNITED STATES PATENTS

|           |         |                 |            |
|-----------|---------|-----------------|------------|
| 2,209,464 | 7/1940  | Loane et al.    |            |
| 2,618,603 | 11/1952 | Schaeffer       | 21—2.5 XR  |
| 2,947,703 | 8/1960  | Larsonneur      | 21—2.5 XR  |
| 3,226,180 | 12/1965 | Irwin           | 21—2.7 XR  |
| 3,260,538 | 7/1966  | Gardner         | 21—2.7 XR  |
| 3,371,010 | 2/1968  | Hamilton et al. | 260—564 XR |

#### OTHER REFERENCES

George Holmes Richter: Textbook of Organic Chemistry, third edition, John Wiley & Sons, New York, 1952 (pp. 280—281 relied on), copy in Group 171.

Herbert H. Uhlig: The Corrosion Handbook, John Wiley & Sons, New York, 1948 (p. 910 relied on), copy in Group 171.

MORRIS O. WOLK, Primary Examiner

35 B. S. RICHMAN, Assistant Examiner

U.S. Cl. X.R.

21—2.5, 58